

## UNITED STATES PATENT OFFICE

2,094,232

## OXIDIZING OF LEAD TO LITHARGE

Robert M. Cole, Bryn Athyn, Pa.

No Drawing. Application August 16, 1933,  
Serial No. 685,424

6 Claims. (Cl. 23—51)

This invention relates primarily to the oxidizing of lead to litharge, but it is also useful in other connections as, for example, in the production of caustic soda and ammonia.

5 The nature, objects and advantages of the invention will appear from the following.

Heretofore, lead has been oxidized to litharge by means of sodium nitrate by a process commonly known as a "dry fusion" in which both the 10 lead and the nitrate are melted and brought into reaction in the fused state. The melting temperature point of lead is 320° C. and of sodium nitrate 316° C.

The present method departs radically from 15 the above procedure in that the oxidation is carried out in a water environment as, for example, in an autoclave. By this new method it is possible to produce litharge and sodium nitrate (as 20 was the case in the known method above referred to) or litharge, sodium plumbite, sodium nitrate, caustic soda and ammonia, and this in almost any desired proportion by varying the conditions 25 as will further appear. This difference between the wet and the dry method is to be attributed to the hydrolysis of sodium nitrate which is a weak salt.

The method is best performed in a forged 30 steel cylindrical autoclave. If the operation is to be conducted without intermittent opening and closing of the autoclave, the latter is set up in a vertical position with bolted, flanged top and bottom, the molten lead and nitrate solutions being admitted through valves in the top plate, and the litharge and aqueous products 35 being withdrawn through similar valves in the bottom plate. Where the operation is to be performed with intermittent opening and closing of the plate, the autoclave is closed at one end and at the other end is provided with a quick opening head. In this case the autoclave is preferably 40 set up in a horizontal position and the charge is carried in a cartridge such as an iron wire mesh basket, preferably of a bore approximating that of the cylinder.

45 1st Procedure.—According to the first procedure, the molten lead is poured through a valve, below which is preferably located a moving or movable screen. The autoclave is partly full of water, and as the fine lead spray produced by 50 the screen strikes the water, there results a

highly surfaced feathered lead. Part of the boiling water is removed, and after closing the lead valve a saturated solution of nitrate of soda at 5 preferably 350° C., is admitted. As the nitrate solution contacts the feathered lead, an exothermic reaction takes place which gradually raises the temperature of the reacting mass to 300° C., 10 325° C., or 350° C., as desired, the pressure ranging from approximately 100 to 200 atmospheres. The temperature is controlled, as for example, by the rate at which the nitrate solution is introduced, or by the concentration of the nitrate solution, or both. The higher the temperature, 15 the shorter the time of the reaction. By control of the temperature, the kind and amount of end products can be accurately determined. As the time is shortened and the temperature increased, the tendency is toward the exclusive production of theoretical amounts of litharge, caustic soda, 20 and ammonia, part of the caustic soda and litharge being united as sodium plumbite. At lower temperatures and longer time, litharge and sodium nitrate alone are produced. The preferred range is from about 280° C. to about 25 350° C.

The solid litharge and caustic soda and ammonia solutions are removed by opening the bottom valves, thus releasing the pressure. Removal may be facilitated by the use of steam and 30 water nozzles situated in the bottom of the autoclave. The erosion and flotation incident to the use of such nozzles readily removes the litharge.

The maximum time necessary is ordinarily approximately thirty minutes.

2nd Procedure.—According to the second procedure the molten lead is poured into one of the cartridges immersed in water in a suitable container mounted in a vertical position, thus producing the feathered lead. The cartridge containing the lead is then slid into the horizontal autoclave in much the same manner as in the loading of a gun. The quick opening head is now closed and the nitrate solution admitted as 40 in the first procedure. When the reaction is 45 over the temperature begins to fall, the head is opened and the cartridge removed.

In the above procedures a slight excess of lead is used in the reaction, but this is readily recovered, remaining in the cartridge or autoclave 50

for re-use. Based on the nitrate, the yield is theoretical for litharge, caustic soda and ammonia, and the process is therefore a useful one as a commercial source for caustic soda and ammonia. 5 The molal heat of the exothermic reaction is two hundred and twenty-nine thousand calories, and therefore quite ample for the evaporation of the caustic soda solution.

Another important advantage and distinction 10 of my process lies in the amount of nitrate of soda required. Whereas the known method required a full molecule of nitrate to furnish sufficient oxygen for an atom of lead, the new method, theoretically, requires only one-fourth of a molecule of nitrate to bring about the same amount 15 of oxidation in the lead, for the reason that due to the water environment there is the following reaction:



20 Because of the oxygen thus made available, a little less than one-third of theory for sodium nitrate is used as contrasted with that needed in the known process.

25 Aside from the appearance of bright new gold which the litharge has while wet, it is also unique in being formed in water in its original state of subdivision in which it may be retained if desired in paste form.

30 Because of the above, and for other reasons, the process is more economic and effective.

With respect to the production of litharge for batteries, the process is particularly useful in that it removes impurities such, for example, as copper 35 and manganese, the presence of either of which in small quantities is detrimental. The copper unites with the ammonia to form a cupro-ammonium solution and the manganese unites with caustic soda, both of which can be removed.

40 The reactions are as follows. The first reaction is—



45 On increase in temperature a second reaction occurs which is as follows:



Adding the first and second reactions the  $\text{NaNO}_2$  cancels out as indicated and we have—



Therefore we have—



showing that one-quarter of the nitrate is required to bring about the same amount of oxidation in the lead.

When the temperature is such that the second reaction takes place there is also, concurrently, a third reaction as follows:



I claim:

1. The process which includes pouring molten lead into water to produce feathered lead, and adding sodium nitrate in the presence of water.

2. The process which includes pouring molten lead into water to produce feathered lead, and adding sodium nitrate in the presence of water, heat and pressure.

3. The process which includes reacting lead and sodium nitrate in a vessel containing water and controlling the temperature to produce caustic soda as an end product.

4. The process which includes reacting lead and sodium nitrate in a vessel containing water and controlling the temperature to produce litharge and sodium plumbite as end products.

5. The process which includes reacting lead and sodium nitrate in a water environment at a temperature of from about 280° C. to about 350° C.

6. The process which includes reacting lead and sodium nitrate in a water environment at a temperature of from about 280° C. to about 350° C. and at a pressure from about 100 to about 200 atmospheres.

ROBT. M. COLE. 45

CERTIFICATE OF CORRECTION.

Patent No. 2,094,232.

September 28, 1937.

ROBERT M. COLE.

It is hereby certified that error appears in the printed specification of the above numbered patent requiring correction as follows: Page 1, first column, lines 18, 20 and 25, and second column, line 23, for "nitrate" read nitrite; and that the said Letters Patent should be read with these corrections therein that the same may conform to the record of the case in the Patent Office.

Signed and sealed this 7th day of December, A. D. 1937.

Henry Van Arsdale,  
Acting Commissioner of Patents.

(Seal)